

## UNITED STATES PATENT OFFICE

2,019,124

## STRIPPING AGENT

John Gwynant Evans and Leslie Gordon Lawrie,  
Blackley, Manchester, England, assignors to  
Imperial Chemical Industries Limited, a corpo-  
ration of Great Britain

No Drawing. Application April 2, 1934, Serial No.  
718,741. In Great Britain April 7, 1933

9 Claims. (Cl. 8—2)

In British Specification No. 400,239 there is described a process for the stripping of textiles dyed with azoic colours comprising the treatment of the dyed materials with a reducing liquor containing an amine or amine salt, one radical in which comprises a straight or branched carbon chain of not less than 10 carbon atoms.

The present invention relates to the stripping of textile fibres dyed with alizarine colours, applied by the usual mordant method, basic colours and vat colours as herein defined.

The invention has for its object the provision of a technically advantageous, economical process of stripping, particularly adapted to the entire or substantially entire removal of solid shades provided by alizarine colours, dyed by the usual mordant methods, basic colours and vat colours.

This object is accomplished according to the invention by treating textile material dyed with the said colours in a liquor containing an amine or amine salt, preferably a quaternary ammonium salt, one radical in which comprises a straight or branched carbon chain of not less than 10 carbon atoms, and also containing where advantageous one or more of the following additional substances, namely, acid, alkali, reducing agent, soluble soap and a sulphonic acid or sulfuric ester as herein defined.

The additional substances may be added or not according to the dye and the textile materials from which it is to be stripped. With basic colours it is usually sufficient to heat in an aqueous liquor with the amine salt or with the amine in a medium containing a little acid. With alizarine colours a reducing agent is usually necessary to give a bath which will reduce the colours. With vat colours an alkali and reducing agent, preferably together with a soluble soap, or a sulphonic acid or sulfuric ester as hereinafter defined is used. When stripping wool and silk and other animal fibres some risk of injury to the fibre is present if alkali is used so alkali is preferably avoided. The acid may be mineral or organic acid. The fibre is stripped white or slightly tinged. In the latter case, for vegetable fibre a supplementary chlorine or chemic treatment may be applied further to improve the ground. In the case of animal fibre a supplementary peroxide treatment is sometimes beneficial.

In stripping in the presence of a reducing agent the amine or amine salts referred to above as well as increasing this degree of stripping also retard the rate of re-oxidation of the reduced dyeings thus giving more even stripped shades, where stripping white is not required.

Suitable amines or amine salts are for example  $\beta$ -di-ethylamino-ethyloleyl amide or its acetate or hydrochloride, heptadecylamine or its hydrochloride (Hoffman, Berichte, 1882, 15, 774) and suitable quaternary ammonium salts are, for example, octadecylpyridinium bromide, cetylpyridinium bromide (cf. British Specification No. 379,396), cetylpyridinium chloride (cf. British Specification No. 392,763), octadecyltrimethylammonium iodide from octadecyl iodide and trimethylamine, cetyltrimethylammonium bromide, cetyltrimethylammonium bromide, cetyltrimethylammonium iodide,  $p$ -stearoamidoethyltrimethylammonium sulphate,  $\beta$ -stearoamidoethyltrimethylamine methosulphate (cf. British Specification No. 294,582) or  $\beta$ -hydroxy-ethyl-N-octadecyl morpholinium bromide (prepared by heating together equimolecular proportions of  $\beta$ -hydroxyethylmorpholine and octadecyl bromide at 140—145° C.).

By vat colours we mean anthraquinone and indigo vat colours and vat colours of the Hydron blue type. By sulphonic acid or sulphuric ester we mean a compound of the class represented by the general formula  $\text{RSO}_3\text{H}$  and  $\text{ROSO}_3\text{H}$  and a soluble salt thereof, where R is an aliphatic saturated or unsaturated radical containing a carbon chain of not less than 10 carbon atoms.

Advantages of our invention are that it provides a ready means of stripping Turkey red and other alizarine mordant colours and vat dyes which are normally very difficult to strip: that it provides a very simple means of stripping basic colours and that all these colours, together with azoic colours can be stripped by the same liquor.

When we speak of dyed textile materials we include also printed textile material but we do not include discharging, that is to say the local removal of colour for the purpose of making coloured patterns.

The following examples in which parts are by weight illustrate but do not limit the invention.

*Example 1.*—A dyeing of Turkey red on cotton is treated for 30 minutes at the boil with 40 times its weight of an aqueous solution prepared by adding 4 parts of caustic soda, 3.75 parts of sodium hydrosulphite and 2 parts of trimethylcetyltrimethylammonium bromide to 1000 parts of water.

The material is stripped to a pale brown shade which can be cleared to a white by treatment for 15—30 minutes in  $\frac{1}{2}$  tw. sodium hypochlorite.

*Example 2.*—A 1% shade of Auramine O (Colour Index No. 655) dyed on tannin mordanted cotton in the usual manner is treated for  $\frac{1}{2}$  hour at the boil in a 0.17% aqueous solution of octa-

decyldpyridinium bromide. The dyestuff is completely removed from the fibre.

*Example 3.*—A 1% shade of Rhodamine 6GBS (Journal of Soc. of Dyers and Colourists, 1933, vol. 49, page 110) dyed on tannin mordanted cotton in the usual way is treated for  $\frac{1}{2}$  hour in a 0.17% aqueous solution of trimethylcetylammmonium bromide. The cotton is stripped to a very pale pink shade.

10 *Example 4.*—As Example 2 but a 1% dyeing of Magenta P (Colour Index No. 677) is treated in a 0.17% aqueous solution of the acetate of the unsymmetrical diethylaminoethylamide of oleic acid. The dyeing is stripped to a very weak bluish red shade.

15 *Example 5.*—A 1% shade of Acronol yellow T (Colour Index No. 815) dyed on silk in the usual manner is treated for  $\frac{1}{2}$  hour at the boil in a 0.17% aqueous solution of trimethylcetylammmonium bromide. The silk is stripped to a very pale yellow shade.

20 *Example 6.*—A 1% shade of Auramine O (Colour Index No. 655) on silk is treated as in Example 5. The dye is almost completely removed from the fibre.

25 *Example 7.*—Cotton yarn dyed with 10% Caledon yellow G (Colour Index No. 1118) is treated for 30 minutes at 90–95° C. with 40 times its weight of an aqueous solution prepared by adding 30 5 parts of caustic soda, 4 parts of sodium hydrosulphite (conc. powder) and 2 parts of benzylidemethylcetylammmonium chloride to 1000 parts of water.

The yarn is stripped to a very pale yellow shade.

30 *Example 8.*—Cotton yarn dyed with 10% Durindone blue 4BC (Colour Index No. 1184) is treated as in Example 7, but using benzylidemethylcetylammmonium sulphonate instead of the quaternary ammonium salt there mentioned.

35 *Example 9.*—The yarn is stripped to a weak blue shade.

40 *Example 10.*—Cotton yarn dyed with 15% Caledon blue R (Colour Index No. 1106) is treated as in Example 7 but using trimethylcetylammmonium bromide as the quaternary ammonium salt.

45 *Example 11.*—The yarn is stripped to a pale blue shade, which, if desired, can be stripped white by treatment for 1 hour in 1° tw. sodium hypochlorite solution.

50 *Example 12.*—Cotton yarn dyed with 10% Caledon jade green paste (Colour Index No. 1101) is treated for 30 minutes at 90–95° C. with 40 times its weight of an aqueous solution prepared by adding 5 parts of caustic soda, 4 parts of sodium hydrosulphite (conc. powder), 0.5 parts of trimethylcetylammmonium bromide and 0.4 parts of oleic acid, to 1000 parts of water.

55 The yarn is stripped to a weak green shade. A similar effect is obtained by substituting textile flakes or cetyl sodium sulphate, or the oleic ester of taurine for the oleic acid.

60 *Example 13.*—Cotton piece goods dyed with 3%  $\beta\alpha$ -naphthothio-indigo are treated for 30 minutes at 90–95° C. with 40 times their weight of an aqueous solution prepared by adding 5 parts of caustic soda, 4 parts of sodium hydrosulphite (conc. powder), 1 part of trimethylcetylammmonium bromide, 0.8 parts of oleic ester of taurine to 1000 parts water.

65 The material is stripped to a white.

70 *Example 14.*—Cotton yarn dyed with 20% Caledon yellow 3G (Colour Index No. 1132) is treated for 30 minutes at 90–95° C. with 30 times its weight of an aqueous solution prepared by adding 2.0 parts of caustic soda, 3.33 parts of sodium hydrosulphite (conc. powder), 0.66 parts

75 of trimethylcetylammmonium bromide and 0.46 parts of palmitic acid to 1000 parts of water.

80 The yarn is squeezed and treated for 15 minutes in  $\frac{1}{2}$ ° tw. sodium hypochlorite solution, followed by a souring treatment with  $\frac{1}{2}$ ° tw. hydrochloric acid. The yarn is stripped to a very weak yellow shade.

85 *Example 15.*—A 20% dyeing of Durindone pink FF. Colour Index No. 1211 on a cotton piece is treated as in Example 12. The material is stripped to a very weak pink shade.

90 *Example 16.*—A 20% dyeing of Caledon jade green (Colour Index No. 1101) on viscose yarn is treated as in Example 6.

95 The material is stripped to a weak green shade.

100 *Example 17.*—A 20% dyeing of Caledon blue RC (Colour Index No. 1114) on viscose yarn is treated as in Example 12.

105 The material is stripped to a weak blue shade.

110 *Example 18.*—Wool dyed a full red with alizarine on an aluminium mordant is treated for 20 minutes at the boil in a solution containing 2 parts of cetyltrimethylammmonium bromide, 2 parts of acetic acid (30%) and 4 parts of sodium formaldehyde sulfoxylate, in 1000 parts of water.

115 It is stripped to a very pale pink colour.

We claim:

1. A process for stripping textile materials dyed with colours selected from the group consisting of alizarine colours, basic colours and vat colours which comprises treating them with a liquor containing a substance selected from the group consisting of amines and amine salts having an aliphatic radical which contains not less than 10 carbon atoms.

2. A process for stripping textile materials dyed with colours selected from the group consisting of alizarine colours, basic colours and vat colours which comprises treating them with a liquor containing a cetyltrialkylammmonium salt.

3. A process for stripping textile materials dyed with colours selected from the group consisting of alizarine colours, basic colours and vat colours which comprises treating them with a liquor containing cetyltrimethylammmonium bromide.

4. A process for stripping textile materials dyed with colours selected from the group consisting of alizarine colours, basic colours and vat colours which comprises treating them with a hot dilute liquor containing cetyltrimethylammmonium bromide.

5. A process for stripping textile materials dyed with vat colours which comprises treating them with a chemically reducing liquor containing a substance selected from the group consisting of amines and amine salts having an aliphatic radical which contains not less than 10 carbon atoms.

6. A process for stripping textile materials with vat colours which comprises treating them in alkaline chemically reducing liquor containing cetyltrimethylammmonium bromide and a soluble soap.

7. A process for stripping materials dyed with vat colours which comprises treating them in alkaline chemically reducing liquor containing cetyltrimethylammmonium bromide and a substance selected from the group consisting of  $RSO_3H$  and  $ROSO_3H$  where R is an aliphatic radical which contains not less than 10 carbon atoms.

75 8. A process for stripping textile materials dyed with alizarine colours which comprises

treating them with a chemically reducing liquor containing a substance selected from the group consisting of amines and amine salts having an aliphatic radical which contains not less than 10  
5 carbon atoms.

9. A process for stripping textile materials

dyed with alizarine colours which comprises  
treating them with a chemically reducing liquor  
containing cetyltrimethylammonium bromide.

JOHN GWYNANT EVANS.  
LESLIE GORDON LAWRIE.